

# UNITED STATES PATENT OFFICE.

WILHELM SCHUMACHER, OF OSNABRÜCK, GERMANY.

## BINDING MEANS FOR BRIQUETS.

1,146,455.

Specification of Letters Patent.

Patented July 13, 1915.

No Drawing.

Application filed July 9, 1913. Serial No. 778,099.

To all whom it may concern:

Be it known at 1, WILHELM SCHUMACHER, chemist, a subject of the King of Prussia, residing at Osnabrück, in the Kingdom of Prussia, German Empire, have invented certain new and useful Improvements in Binding Means for Briquets, of which the following is a specification.

In connection with the production of briquets and particularly such as are made of finely divided substances such as coal dust or iron ores, it has been frequently suggested that tar (coal tar) be employed as the binding means. Briquets thus made when baked together have not proved practicable for the reason that the tar melts when heated, becoming quite fluid at the higher temperatures, thus causing the briquets to disintegrate and to return to their condition as powdered substances. The binding capacity of tar is totally lost in the presence of heat.

I have now discovered that the defects which were inherent in connection with the use of tar can be obviated by the employment as a binding means of wood-tar in place of ordinary tar and if simultaneously there is added a small proportion of hydrate of lime. Five per cent. of wood-tar and one per cent. of lime is a fair average example of the proportion of the binding ingredients. If these substances thus specified are employed a reaction seems to take place between the lime and the components of the

wood-tar which apparently results in the creation of insoluble compounds. The briquets produced by the use of this binding means are far more solid than the briquets made by the use of tar alone and they retain, even in the presence of great heat, their shape and condition as briquetted material. Calcium hydroxid or hydrate of lime which has been suggested as a binder for ores and the like does not result in anything like the rigidity or solidity in the briquets such as is produced by a mixture of wood-tar and calcium hydrate as described by me. Ordinary tar, that is coal tar, does not possess the property of hardening or of producing a hardened condition when mixed with lime.

What I claim is:

1. Binding means for briquets of finely powdered substances such as coal or ores, consisting of wood-tar and calcium hydrate.
2. Binding means for briquets of finely powdered substances such as coal or ores, consisting of wood-tar and calcium hydrate in the approximate proportions of five per cent. of wood-tar and one per cent. of calcium hydrate.

In testimony whereof, I have hereunto set my hand in the presence of two subscribing witnesses.

WILHELM SCHUMACHER.

Witnesses:

HENRY HASPER,  
WOLDEMAR HAUPT.